

H. L. DOHERTY.

METHOD OF CARBONIZING COAL AND OBTAINING GAS.

APPLICATION FILED NOV. 15, 1911. RENEWED APR. 28, 1916.

1,187,050.

Patented June 13, 1916.

2 SHEETS—SHEET 1.



H. L. DOHERTY.

METHOD OF CARBONIZING COAL AND OBTAINING GAS.  
APPLICATION FILED NOV. 15, 1911. RENEWED APR. 28, 1916.

1,187,050.

Patented June 13, 1916.

2 SHEETS—SHEET 2.



Witnesses:

Wm. H. Blackman  
Frank L. Blackman  
H. A. Mackenzie

Henry L. Doherty Inventor  
By his Attorney Frank S. Young.

# UNITED STATES PATENT OFFICE.

HENRY L. DOHERTY, OF NEW YORK, N. Y.

## METHOD OF CARBONIZING COAL AND OBTAINING GAS.

1,187,050.

Specification of Letters Patent. Patented June 13, 1916.

Application filed November 15, 1911, Serial No. 660,451. Renewed April 28, 1916. Serial No. 94,276.

To all whom it may concern:

Be it known that I, HENRY L. DOHERTY, a citizen of the United States, and resident of New York city, in the county of New York and State of New York, have invented certain new and useful Improvements in Methods of Carbonizing Coal and Obtaining Gas, of which the following is a specification.

10 My invention relates to methods of carbonizing coal and obtaining gas, and, in particular, to a method of carbonizing coal in a shaft furnace.

15 The object of my invention is to provide a method of carbonizing fuel which will permit the carbonization of the fuel in a shaft furnace by heat developed in the shaft furnace itself and at the same time to take off all the products of the carbonizing operation.

20 This application discloses matter which I do not claim specifically herein but do claim in my applications Ser. Nos. 660450 and 660453, filed Nov. 15th, 1911.

25 To this end my invention, briefly stated, comprises the charging of bituminous fuel into a shaft furnace, the establishing of a region of localized and limited combustion in the interior of said fuel mass by introducing a carefully regulated volume of air thereinto, whereby a relatively short middle section or portion of the fuel mass in the said shaft is raised to a carbonizing temperature, withdrawing the gaseous products 30 of the carbonization through the relatively cold fuel mass in the upper portion of the said shaft, whereby the sensible heat of the gases discharging from the carbonizing zone is absorbed by the said cold fuel, deluminating a portion of the said gas, saturating the same with water vapor, and conducting the vapor laden deluminated gas to the lower part of the said shaft furnace and passing it upward through the mass of coke filling 35 the same. This coke, of course, discharges from the carbonizing zone at a comparatively high temperature. By properly proportioning the relation between the volume of the vapor and deluminated gas returned 40 to the shaft and the heat held by the coke filling the part of the same below the carbonizing zone, it is possible to cool the coke discharged down to practically atmospheric temperature. Besides the above, my invention embodies various other features which 45 will more fully appear later.

In the accompanying drawings I have shown a form of apparatus comprised in and suitable for carrying out my invention.

Figure 1 is a vertical cross-section through the carbonizing furnace on line A—B of Fig. 2. Fig. 2 is a plan of the apparatus. Fig. 3 is a vertical section similar to Fig. 1 but showing the apparatus for discharging the coke and transporting the same. Fig. 4 60 is a front elevation of the bottom of the furnace. Fig. 5 is a vertical cross-section through the water evaporator.

1 refers to the carbonizing furnace as a whole, 2 indicates the carbonizing region of 70 the same, 3 indicates the preheating region, and 4 the coke cooling region. The portion of the shaft 1 indicated by the numerals 2 and 3 is, in reality, a single chamber and there is no fixed line of demarcation between 75 the two regions. The upper boundary of the carbonizing region, designated by 2, depends simply upon the position of the isotherm of the lowest temperature at which distillation will take place with the variety 80 of coal used, and fluctuates also with the operating condition of the furnace at any given time.

5 is a continuous discharging device, 6 is 85 a continuous charging device.

7 is a blower for supplying the air to support the combustion in 2.

8 is a deluminator. 9 an ammonia scrubber. 10 an exhauster withdrawing the gases 90 from the preheating chamber 3 and forcing them to the purifying train.

11 is the gas off-take. 12 the gas conduit to the purifying train.

13, 13, etc., are poke-holes provided for purposes of observation and manipulation 95 of the charge.

14 is the connection from the gas main 12 to the deluminator 8.

12' and 14' are valves on, respectively, 12 and 14 to regulate the distribution of the 100 gas between the purifiers and the deluminator.

15 is the connection from the evaporator 25 to the coke cooling chamber 4 of the furnace.

16 is the air connection from the blower 7 to the air bustle-pipe 26.

17 designates the air inlets to the carbonizing chamber from the bustle-pipe 26.

18 is a screen or grizzly for screening out 110 the fines from the coke discharged from the cooler.

- 19 is the ash door permitting the removal of ash from the ash pit 36 of the furnace. 20 is the discharge chute from screen 18. 21 is the adjustable vane regulating the 5 distribution of the screened coke between the chutes 22 and 32. 23 and 33 are coke conveyers, one conveying the coke to the place of storage and the other elevating a portion of the coke to the 10 bin 34. 25 is the evaporator and recuperator for loading the gas returned to the cooling chamber 4 with water vapor. 27 is the connection from the ammonia 15 scrubber 9 to the evaporator 25. 28, 28, etc., are the water distributers of 25, while 30 is the water supply pipe to 25, having the valve 29. 31, 31, etc., are the tubes of 25. 20 35 is the coal conveyer which carries the coal to bin 34. 37 is an air connection from the main air line to the bottom of the cooler 4. 37' is a valve on 37. 25 38 is a manhole provided in the cover of the shaft. In starting operations, coke is fed into the shaft of the furnace 1 until the same has been filled to approximately the lower limit 30 of the carbonizing chamber. Kindling is now charged upon the coke and the shaft filled to the top with a mixture of raw coal and coke. The kindling is now ignited by inserting a torch through one of the pock-holes 13. Air is supplied to the carbonizing chamber under low pressure by the blower 7. At first, the supply of air must be rather large since a large amount of heat is required to heat up the walls of the furnace 40 and the mass of cold fuel in the middle portion of the charge. When the combustion chamber and the fuel column have been raised to the proper carbonizing temperature, the air is gradually 45 cut down until only a sufficient quantity is being used to maintain the carbonizing chamber at the proper temperature. The gas from the combustion, the gases and vapors evolved from the coal and the gas introduced at the bottom of the furnace pass 50 upward through the preheating chamber 3 in contact with the fuel charge filling the same. In contact with the comparatively cold fuel in the upper part of the shaft the 55 gases are cooled down to a temperature which depends upon the quantity of sensible heat carried by the gases in relation to the heat capacity of the fuel mixture charged, between the temperature at which it is introduced and the temperature prevailing 60 in the carbonizing chamber. As a rule the gases will discharge from the preheater 3 at a temperature of between 212° F. and 300° F. When this is the case, the larger 65 part of the tarry vapors carried by the gas

from the carbonizing zone is condensed on the relatively cool fuel in the preheater. The outgoing gas therefore usually carries substantially only the lighter condensable hydrocarbons of the distillation products of the coal, such as benzol and allied products and water vapor. The temperature of the withdrawn gases should not be permitted under any circumstances to exceed the boiling or condensing temperature of the pitch-forming bodies. 70 75

Under the action of the exhauster 10, the gases are drawn off from the upper part of chamber 3 through the pipe 11, passing in the arrangement of apparatus shown, 80 through the intertubular space of the evaporator 25, where they deposit their water vapor and some of the more easily condensed hydrocarbons, and thence to the exhauster 10. Discharging from 10 the gases 85 divide into two streams. One stream passes through the pipe 12 to the ordinary purifying train and thence to a holder in the usual course. The second stream passes through the passage 14 to the deluminator 8, 90 where it is scrubbed with oil which absorbs the major portion of its illuminants. Thence the deluminated gas passes through the pipe 24 to the ammonia scrubber 9, where its ammonia and some of its other 95 constituents are removed. Valves 12' and 14' regulate the distribution of the gas between the deluminator 8 and the main purifiers. From 9 the deluminated and ammonia-free gas passes through the connection 100 27 to the evaporator 25.

The evaporator 25 is simply a tubular heater, the upper ends of the tubes having inserted in them distributers, 28. A small depth of water is maintained on the upper 105 tube sheet by regulating the valve 29 on the water pipe 30. The water is permitted by the distributers to flow onto the interior surfaces of the tubes as a thin film. Passing down through the tubes, the water is heated 110 by the moderately hot gases coming from the preheating chamber 3 which, as before explained, pass upward through the intertubular space. The gas from the ammonia scrubber 9 flows through the pipe 27 and 115 enters the evaporator 25 above the upper tube sheet. Passing down through the tubes, 31, the gas is heated by contact with the water flowing down the inside of the tubes and at the same time takes up a portion of 120 the water.

By properly regulating the velocity of the gas through the tubes 31, the gas will be caused to discharge from 25 either practically or completely saturated with water 125 vapor. Usually the returned gas will enter the cooler 4 through the conduit 15 at approximately 200° F. At this temperature the returned gas will carry about six times its own weight of water vapor. Entering 130

the cooler 4, the vapor-laden gas ascends through the furnace shaft in contact with the descending coke, taking up the heat of the latter and carrying it back into 5 the carbonizing chamber 2. By properly proportioning the volume of the gas-vapor current introduced into 4 it is possible to cool the coke down to practically the temperature at which the gas is introduced into 10 4. It is desirable, however, that no more gas and vapor should be introduced into 4 than is required to accomplish this cooling.

Besides its cooling action in 4, the water vapor introduced markedly increases the 15 yield of gas. This is accomplished not so much through its own dissociation into hydrogen and oxygen (with the combustion of the latter to CO), as by the influence which it exerts in assisting in the liberation 20 of the volatile matter from the coal. Usually in gas house practice the coke will retain upward of 5% volatile matter, in spite of the fact that it has been exposed for hours to a comparatively high temperature. By introducing steam into the retorts, during the last part of the carbonizing period, by far the greater part of this residual volatile matter is liberated. In the same way, the presence of the water vapor assists 25 in freeing the coke from volatilizable matter and thus increases the yield of gas. While in the lower portion of the carbonizing zone some little dissociation of water vapor may take place with the liberation of H and CO, 30 this reaction does not proceed to any great extent owing to the fact that the atmosphere of the furnace, at the locality where the temperature would ordinarily be high enough to bring about reaction between the 35 carbon of the coke and the water vapor, contains a large percentage of hydrogen and carbon-monoxid owing to the distillation and combustion taking place. This high partial pressure of both the H and CO acts 40 to retard the reaction between carbon and H<sub>2</sub>O and to increase the temperature required to bring it about.

The cold coke, together with the slight amount of ash which is formed by the limited combustion taking place in 2, is discharged either continuously or intermittently from the bottom of 4 by operating the mechanical discharging sealing device, 5. This is in effect simply a drum having a 55 number of longitudinal pockets, and working in a cylindrical casing. The casing is longitudinally slotted at the top and bottom to provide passage for, respectively, the admission and discharge of the coke. The 60 seal 5 is really a provision against the loss of the gas introduced into 4 through 15 rather than against the admission of air. The speed of operation of 5, and consequently the rate of discharge of the coke, 65 is so regulated that the charge is caused to

settle through the carbonizing chamber 2 at a rate corresponding to the rate of carbonization. In other words, the charge should be caused to move through 2 at such a rate that the raw coal in the fuel mixture will have been completely carbonized (or rather, 70 will have been carbonized to the extent desired) by the time that it has passed below the air inlet 17. The rate of carbonization for any given mixture of coal and coke with- 75 in the limits of the capacity of the apparatus depends simply upon the rate at which the air is supplied by blower 7 through 16. It is therefore possible to quickly adjust the make of gas to the demand by simply vary- 80 ing the air supply. The rate of drawing must of course be varied also, but since this depends almost entirely upon the rate at which air is supplied it is simply a function of the air supply and is fixed by the 85 latter.

The ratio of air required to coal carbonized will vary greatly with different coals according to the heat required to carbonize them. It has been determined experimentally that the actual heat of carbonization in the case of coals experimented upon varied from the development of 779 B. T. U. per pound of coal down to an absorption of 90 about 168 B. T. U. per pound. The experimental results would seem to indicate that the heat developed in the carbonization varied directly as the oxygen contents of the raw coal. With a coal giving the first result, by my method of carbonization, the operation, after once being started, will be self-supporting, since in this case it is only necessary by my method to supply an amount of heat equivalent to the radiation and conduction losses. This would, in the case of 95 the coal referred to, be nearly or, possibly, entirely supplied by the heat evolved in the carbonizing of the coal. With such a coal the quantity of air supplied would, under normal conditions be *nil*. 100

As stated above, the composition of gas coals and the results which they give on carbonization are so variable that it is impossible for me to here prescribe a specific 115 ratio of air to coal that would be applicable in all cases. I may say that, in general, I aim to use the minimum quantity of air that will generate the quantity of heat required in the carbonization of the particular coal used. 120

The combustion taking place in 4 will be localized and will occur in the immediate vicinity of the air inlet 17 and for a short distance upward in the charge. The maximum temperature therefore occurs at the 125 bottom of the carbonizing zone. The hot gases from the combustion ascend through the fuel column occupying the chamber, carrying the heat of the combustion up into the portion of the charge undergoing car- 130

bonization. By thus generating the heat required in the body of the carbonizing material in immediate contact with the same I am able to secure a high utilization of the heat generated. Besides, owing to the actual contact of the combustion gases with the fuel the required temperature to be produced by the combustion is comparatively low—not necessarily higher than the maximum temperature actually required for completing the carbonization—say 1500° F. In the combustion zone, however, the temperature is usually unavoidably higher than this, although I aim to so regulate the introduction of air and the flow of gas from the cooler 4 that the maximum temperature of the combustion will be brought as low as practicable.

In ordinary practice in coal carbonization the heat for carbonizing the coal is transmitted to the latter through comparatively thick walls of fire clay. In this case, it is absolutely essential that a high temperature should be developed in the combustion flues (about 2400°) in order to secure a sufficiently great temperature difference between the two sides of the wall to drive the heat through it with sufficient rapidity. The high temperature of the combustion in this case unavoidably occasions a much higher rate of loss by radiation than occurs with the low temperature used by me. In addition, the manner in which I conduct the combustion by my method enables me to carry on the same in a chamber easily provided with thick walls of heat insulating material. For these reasons, I am able to reduce the radiation and conduction losses from my apparatus to a minimum.

Owing to the fact that (as explained in detail below) I preferably introduce a stream of treated combustible gas from the furnace itself, together with a larger volume of water vapor, into the lower part of the same and cause it to traverse the full height of the shaft, the air introduced is mixed with this gas as soon as it enters the shaft. The initial combustion, therefore, is partly with the combustible gas and partly with the coke of the charge. The comparatively large proportion of water vapor present, however, tends markedly to reduce the reaction between the air and gas.

The heat developed by the combustion taking place in the lower portion of the carbonizing chamber is communicated not only to the combustion products but the coke in the immediate vicinity of the combustion and the distillation gases from the charge. The temperature produced, therefore, is much below that which would theoretically be due to the combustion in an undiluted atmosphere by the quantity of air introduced. Since, however, the gases from 4 enter 2 at approximately the temperature of

the coke discharging from the same, the temperature of the mixed gases from the lower part of 2 will be somewhat higher than that actually required for the carbonization. These hot gases ascend through the carbonizing chamber 2, giving up their heat to the descending column of mixed coal and coke. As they pass upward the gases become cooler and cooler until they fall below the minimum temperature required for carbonization. Above the level at which they reach this temperature their further cooling is due to the evaporation of moisture from the coal and to the transfer of their heat to the cold coal.

In passing through the upper part of the furnace shaft the gases from the carbonizing zone are deprived by condensation of such of the condensable vapors which they carry as are condensable at the temperature prevailing at 3. With the usual proportion of gases to fuel the gases will nearly always leave the preheating chamber 3 somewhat above 212° F., or at least above that temperature at which water will be deposited. They will therefore deposit on the coal nearly all of the tar-forming and other condensable constituents which they carry save such easily vaporizable substances as water vapor, benzol and allied compounds. This tarry matter will be, to some extent, absorbed in the pores of the coke which forms a portion of the charge and thus be slowly carried down and, in part, run down through the interstices of the charge as liquid into the hotter regions of the furnace, where the tar will be, in part, vaporized to be again condensed and carried down and, in part, converted into permanent gas. This operation is repeated, the tar always reaching on its downward trip a hotter region of the furnace than that in which it was originally vaporized, until it has become wholly converted into permanent gas, with the exception of the heavy pitch and free carbon formed in its gasification. This latter is deposited in the coke formed, adding materially to its density and increasing its hardness.

The comparatively cool gas drawn off from the furnace through 11 by the exhauster 10, as before stated, is divided into two streams, one passing to the regular purification train, while the other, after the removal of most of its illuminants and its ammonia, is saturated with water vapor in 25 and introduced into the bottom of the coke cooler 4. The volume of this returned gaseous stream is, as before explained, to be fixed by that which is required to absorb the sensible heat carried out of 2 by the coke. The volume of the circulated gas, therefore, will depend upon the proportion of coke introduced with the raw coal as well as upon the temperature at which the gas discharges

from the furnace, since upon this temperature depends to a great extent the quantity of water vaporized. Since this latter will vary with different coal the proportion of the returned gas to the distillation gas will vary likewise. Usually it will vary from  $\frac{1}{4}$  to  $\frac{1}{2}$  of the latter when it is returned saturated with water vapor.

The coke may be discharged through 5 either intermittently or continuously. Continuous discharging is preferable as it gives more uniform operating conditions. The discharged coke, mixed with a very small proportion of ash, falls onto the grizzly 18. 15 In passing over this the fine material is screened out and may be raked out of the door 19. The screened coke discharges from 18 through the chute 20 and is divided by the adjustable cone 21 into two 20 streams—one going through the chute 22 to the conveyer 23, which carries it to the place of storage, while the other passes through the chute 32 onto the conveyer 33 which elevates it to the bin 34. A conveyer, 35, discharges into the bin 34 the proper proportion 25 of raw coal to form the proper charge mixture.

The relation between the coke and raw coal to be used in the charge mixture will 30 vary with the kind and quality of the coal. With a highly caking coal the proportion of coke in the mixture may be in extreme cases run to more than double that of the coal. Ordinarily, however, it will run from one- 35 third of to about equal to the weight of the raw coal.

The function of the coke in the mixture is to maintain the charge column in the shaft 40 of the furnace in a condition that will permit a free flow of the gas current through it. In an apparatus of the kind that I prefer to use it is of the highest importance that the fuel bed be maintained free and open to the blast, since with the high charge column 45 that I prefer to use the resistance to the passage of the draft would otherwise be prohibitive. By properly proportioning the mixture, this end can be secured without difficulty. Owing to the practically complete recuperation 50 of the heat of the coke before the latter is discharged, which I secure, no loss in heat economy results from this use of the coke to dilute the raw coal.

It is to be understood that I do not limit 55 myself to the use of a portion of the gas from the furnace itself for the purpose of recuperating the heat of the coke in the present process. It is obvious that I may substitute combustion gases for the deluminated gas as the carrier for the water vapor, or any other suitable gas, without affecting the underlying principles of my invention, which are, simply, the returning to the carbonizing apparatus of the heat carried away 60 from it by the discharged products and the

making up any deficiency in the heat below that required to maintain the carbonizing operation by establishing a limited combustion in the said carbonizing chamber. Even steam alone may be substituted for the mixture of permanent gas and water vapor 70 which is my preferred cooling medium.

While I prefer to introduce the air into the furnace at the lower part of the carbonizing zone as described, I may in some cases 75 (particularly where I am using combustion gas and water vapor, or steam alone, as the medium for recuperating the heat of the coke) introduce the air into the bottom of the cooler together with the cooling draft 80 current. In this case the valve 16' is closed and valve 37' on connection 37 opened. The advantage of this is that I thus utilize the air introduced in recuperating the heat of the coke and can by so much reduce the 85 volume of gas and vapor introduced through 15.

An important feature of my invention is that I am able to exercise a very effective regulation of the make of gas by simply 90 varying the rapidity of feed of the air and fuel. I can even make this control of the air automatic by a suitable balanced pressure device connected on the one hand with the trunk main and on the other with either 95 a governor regulating the speed of the blower 7, or with a throttle valve on 16. In the latter case a relief valve, 38', is placed on the air line 16, and the blower may be run at constant speed. Owing to the possibility 100 of this automatic regulation of the make of gas I am able to dispense with the customary holder and connect the outlet of the purifying system directly with the trunk main. Since the holder usually represents a large 105 portion of the investment for a gas works, the economic advantage of my invention from the investment standpoint is marked, aside from the economies in operation which I am, thereby, able to secure.

A great advantage of my invention is that the "standby" losses are very light, while, at the same time, the apparatus may be quickly brought up again to maximum capacity of output. During a "shut-down" it is only 115 necessary to supply sufficient air to the fuel in the carbonizing chamber to generate enough heat to balance the radiation losses from the shell of the apparatus. In this case the manhole 38 at the top of the furnace 120 may be opened and the gases permitted to escape into the atmosphere.

It is to be understood that while I have shown a vertical shaft for carrying out my process, I do not limit myself to carrying 125 out my invention with a vertical fuel body. Instead I may work with a horizontal or inclined fuel body. It is advantageous, however, to work with a fuel body which is maintained on an incline above the natural angle 130

of repose of the fuel mixture, so that the fuel body will be advanced through the fuel conduit by gravity as portions of the fuel body are removed from the bottom of the same. There are particular advantages in maintaining the fuel body substantially vertical, one of which is the greater uniformity of draft distribution which may thereby be secured.

10 It is to be understood that the word "inclined", as I use it in the following claims, refers to any position of the fuel body not horizontal.

Having described my invention, what

15 I claim is:

1. The steps in the manufacture of coke and gas which comprise, producing a relatively long advancing body initially comprising coal mixed with sufficient compara-

20 tively coarse coke to maintain said advancing body permeable to gases generated therein, said advancing body having a localized zone of intense heat at a midpoint and being relatively cool and externally un-

25 heated at the charging end and at the withdrawal end, and supplying air to said zone of intense heat to keep up the temperature therein and produce coking of the coal, the amount of air so supplied being merely

30 that necessary for such maintenance.

2. In the manufacture of coke and gas the process which comprises, producing a relatively long advancing body initially composed of coal and coke having a localized

35 zone of intense heat at a midpoint of sufficient length to coke said coal and being relatively cool at the charging end and at the withdrawal end, maintaining the heat in said zone by injection of sufficient com-

40 bustion-producing gas for maintenance of said heat with withdrawal of gaseous products of the action, withdrawing cool coke, diverting a portion of the withdrawn coke, admixing the remaining coke with fresh

45 coal and charging the mixture to form said advancing column.

3. The process of continuously carbonizing bituminous fuel to produce gas and carbonized fuel which comprises, producing a

50 relatively long advancing body initially composed of fresh fuel and carbonized fuel in regulated proportions, said body having a localized region of coking temperature at a midpoint and being relatively cool at the charging end and at the withdrawal end, injecting into said localized region merely

55 enough air to maintain a coking temperature therein, withdrawing cool carbonized fuel, mixing a regulated portion of the

60 withdrawn carbonized fuel with fresh fuel, the proportion of carbonized fuel in the mixture being that required to maintain the said fuel body in a condition permitting free passage of the draft current there-

65 through by preventing the formation of

large aggregates due to the caking of the fresh fuel, and charging the mixture to form said advancing body.

4. The process of manufacturing gas and carbonized fuel which comprises, producing a relatively long advancing body initially composed of fresh fuel and carbonized fuel in regulated proportions, said body having a localized zone of coking heat at a midpoint and being relatively cool at the charging end and at the withdrawal end, maintaining the heat in said zone by injection of combustion-supporting gas in the amount necessary for such maintenance, withdrawing cool carbonized fuel, mixing a regulated portion of the withdrawn carbonized fuel with fresh fuel, the proportion of carbonized fuel in the mixture being that required to maintain the said fuel body in a condition permitting free passage of the draft current therethrough by preventing the formation of draft-obstructing aggregates due to the caking of the fresh fuel in the fuel body, and charging the mixture to form said advancing body.

5. The process of manufacturing gas and carbonized fuel which comprises, producing a relatively long advancing body initially composed of a mixture of fresh fuel and carbonized fuel in regulated proportions, said body having a localized region of coking temperature at a midpoint and being relatively cool at the charging end and at the withdrawal end, maintaining the temperature in the said zone by injection of

95 sufficient combustion-producing gas for that purpose with withdrawal of gaseous products of the action, withdrawing cool carbonized fuel, mixing a regulated portion of the withdrawn carbonized fuel with fresh

100 fuel, the proportion of carbonized fuel in the mixture being that required to maintain the said fuel body in a condition permitting free passage of the draft current therethrough by preventing the formation

105 of draft-obstructing aggregates by the caking of the fresh fuel in the fuel body, and charging the mixture to form said advancing body.

6. In the manufacture of carbonized fuel and gas the process which comprises, producing a relatively long advancing body initially composed of a mixture of fresh and carbonized fuel, maintaining a localized

110 carbonizing temperature in an intermediate section of said fuel body, by injecting air in the amount necessary for that purpose, introducing into that portion of said fuel body which has advanced beyond

115 the region of carbonizing temperature a draft current of relatively cool gaseous fluid, to quench the carbonized fuel in said portion of said fuel body and to heat said

120 current, withdrawing the cooled carbonized fuel, rejecting a portion of said carbonized

125 fuel, the proportion of carbonized fuel in the mixture being that required to maintain the said fuel body in a condition permitting free passage of the draft current therethrough by preventing the formation of

130 draft-obstructing aggregates due to the caking of the fresh fuel in the fuel body, and charging the mixture to form said advancing body.

fuel, mixing the remainder with fresh fuel to maintain the permeability to gases of said advancing body in said region of carbonizing temperature, and charging the 5 mixture to form said advancing body.

7. In the manufacture of coke and gas the process which comprises, producing a relatively long advancing body composed initially of coal and coke, said body having an 10 intermediate localized zone of coking temperature at a mid-point and being relatively cool at the charging end and at the withdrawal end, maintaining the heat in said zone by injection of sufficient combustion- 15 supporting gas for that purpose, introducing into the withdrawal end of said body a draft current of relatively cool gaseous fluid and conducting said fluid through said body in a direction opposite to the direction of 20 advance of said body to quench the coke in that portion of said body which has advanced beyond the said zone of coking temperature and to heat said gaseous fluid, withdrawing the cooled coke, admixing a 25 regulated portion of the coke withdrawn with fresh coal, and charging the mixture of coke and fresh coal to form said advancing body.

8. In the manufacture of carbonized fuel 30 and gas the process which comprises, producing a relatively long advancing body composed initially of fresh and carbonized fuel, said body having an intermediate localized zone of carbonizing temperature, 35 and being relatively cool at the charging end and at the withdrawal end, maintaining the carbonizing heat in said zone by injection of sufficient combustion-supporting gas for that purpose, introducing into the withdrawal 40 end of said body a draft current of relatively cool gaseous fluid to quench the carbonized fuel in that portion of said body which has advanced beyond the zone of carbonizing temperature and to heat the said 45 gaseous fluid, withdrawing the cooled carbonized fuel, admixing a regulated portion of the withdrawn carbonized fuel with fresh fuel, the proportion of carbonized fuel in 50 said mixture being that required to maintain the said fuel body in a condition permitting free passage of the draft current therethrough by preventing the formation of draft-obstructing aggregates by the caking of the fresh fuel in the fuel body, and 55 charging the so-formed mixture to form said advancing body.

9. In the manufacture of carbonized fuel and gas the process which comprises, producing a relatively long advancing body 60 composed initially of fresh and carbonized fuel, said body having an intermediate localized zone of carbonizing temperature and being relatively cool at the charging end and at the withdrawal end, maintaining the 65 carbonizing temperature in said zone by in-

jection of sufficient combustion-supporting gas for that purpose, introducing into the withdrawal end of said body a draft current of relatively cool gaseous fluid to quench the carbonized fuel in that portion of said 70 body and to heat the said gaseous fluid, the volume of said gaseous fluid being that required to cool the said carbonized fuel to the desired degree, withdrawing the cooled carbonized fuel, mixing a portion of the withdrawn carbonized fuel with fresh fuel, the proportion of carbonized fuel in the mixture being that required to maintain the said fuel body in a condition permitting free 75 passage of the draft current therethrough by preventing the formation of draft-obstructing aggregates by the caking of the fresh fuel in the fuel body, and charging the so-formed mixture to form said advancing 80 body.

10. In the manufacture of coke and gas the process which comprises, producing a relatively long advancing body of carbonized and bituminous fuel having a localized zone of carbonizing temperature at a midpoint and being relatively cool at the charging end and at the withdrawal end, maintaining the carbonizing temperature in said zone in part by injection of sufficient combustion-supporting gas for that purpose 95 and in part by returning to said zone the major part of the heat carried out of the same by the hot gases withdrawn from said zone, the return of said heat being effected by contacting the withdrawn gases with the portion of said body advancing toward said zone to preheat said portion of said body and to cool and purify said gases, withdrawing cooled carbonized fuel, mixing a portion of the withdrawn coke with fresh 100 bituminous fuel, and charging the mixture 105 to form said body.

11. In the manufacture of carbonized fuel and gas, the process which comprises producing a relatively long advancing body 110 composed initially of carbonized and bituminous fuel, said body having an intermediate zone of carbonizing temperature at a midpoint and being relatively cool at the charging end and at the withdrawal end, maintaining the carbonizing temperature in said zone in part by injection of sufficient combustion-supporting gas for that purpose and in part by returning to said zone the major part of the heat carried 115 out of the same by the hot gases, the return of said heat being effected by withdrawing hot gases from said zone, contacting the withdrawn gases with the portion of said body advancing toward said zone to preheat 120 said portion of said body and to cool and purify said gases, contacting with that portion of said body which has advanced beyond said zone in counter-current relationship a current of gaseous fluid to quench 125 130

the carbonized fuel in the said body and to heat said fluid, withdrawing the cooled carbonized fuel, mixing a regulated portion of the coke withdrawn with bituminous fuel, and charging the mixture of carbonized and bituminous fuel to form said advancing body.

12. In the manufacture of carbonized fuel and gas the process which comprises, producing a relatively long fuel body composed initially of carbonized and bituminous fuel, said body having an intermediate localized zone of carbonizing temperature, and being relatively cool at the charging end and at 15 the withdrawal end, maintaining the carbonizing temperature in said zone in part by injection of sufficient combustion-supporting gas for that purpose and in part by returning to said zone the major part 20 of the heat carried out of the same by the hot gases, the return of said heat being effected by withdrawing hot gases from said zone, contacting the withdrawn gases with the portion of said body advancing toward 25 said zone to preheat said portion of said body and to cool and purify said gases, contacting with that portion of said body which has advanced beyond said zone a current of gaseous fluid to quench carbonized 30 fuel of said portion of said body and to heat said fluid, withdrawing the cooled carbonized fuel, admixing a regulated portion of the withdrawn carbonized fuel with bituminous fuel, the proportion of carbonized 35 fuel in said mixture being that required to maintain said fuel body in a condition permitting free passage of the draft current therethrough by preventing the formation of draft-obstructing aggregates by 40 the caking of the bituminous fuel in the fuel body, and charging the so-formed mixture to form said advancing body.

13. In the manufacture of carbonized fuel and gas the process which comprises, producing a relatively long advancing body composed initially of bituminous fuel and carbonized fuel, said body having an intermediate localized zone of carbonizing temperature and being relatively cool at the 45 charging end and at the withdrawal end, maintaining the carbonizing temperature in said zone by injection of sufficient combustion-supporting gas for that purpose and by preheating the fuel before introducing 50 the same into said zone, said fuel being preheated by withdrawing hot gases from said zone, contacting said gases with that portion of said body advancing toward said zone to preheat said portion of said body 55 and to cool and purify said gases, contacting with that portion of said body which has advanced beyond said zone a current of gaseous fluid to quench the carbonized fuel of the said body to the degree desired and 60 to heat said fluid, withdrawing cooled car-

bonized fuel, admixing a regulated portion of carbonized fuel with bituminous fuel, the proportion of carbonized fuel in the mixture being that required to maintain the said fuel body in a condition permitting 70 free passage of the draft current therethrough by preventing the formation of draft-obstructing aggregates by the caking of the fresh fuel in the fuel body, and charging the mixture of carbonized and 75 fresh fuel to form said advancing body.

14. In the manufacture of coke and gas the process which comprises, producing a relatively long fuel body of mixed coal and coke in regulated proportions, said fuel 80 body being relatively cool at the charging end and at the withdrawal end, the proportion of coke in the said mixture being that required to prevent the formation of draft-obstructing aggregates through the caking 85 of the coal of said mixture and so to maintain the fuel body in a condition permitting free passage of the draft therethrough, advancing said fuel body through a comparatively long conduit, maintaining a carbonizing 90 temperature in an intermediate localized carbonizing region of the said fuel body to decompose bituminous matter of the fuel of said body, to form gas, condensable vapors and carbonized fuel, the said carbonizing temperature being maintained by introducing a limited and regulated quantity of combustion-supporting draft current 95 sufficient for the stated purpose into the said fuel body in said region, withdrawing gases 100 from the upper part of said fuel body, withdrawing cooled carbonized fuel from the lower part of said fuel body, mixing a regulated portion of carbonized fuel with bituminous fuel, and charging the mixture 105 onto the upper part of said fuel body.

15. In the manufacture of coke and gas the process which comprises, producing a relatively long fuel body of mixed coal and coke in regulated proportions, said body 110 being relatively cool at the charging end and at the withdrawal end, the proportion of coke in said mixture being that required to prevent the formation of draft-obstructing aggregates through the caking of the coal of said mixture and so to maintain the fuel body in a condition permitting free passage of the draft therethrough, advancing said fuel body through a comparatively long conduit, maintaining a carbonizing temperature in an intermediate localized carbonizing 115 region of the fuel body to decompose bituminous matter of the fuel of said body, to form gas, condensable vapors and carbonized fuel, the said carbonizing temperature being maintained by introducing a limited and regulated quantity of combustion-supporting draft current sufficient for the stated purpose 120 into the said fuel body in said carbonizing region, withdrawing gases 125 and

vapors from said carbonizing region, conducting the gases and vapors withdrawn from said carbonizing region through the portion of said fuel body above said region to heat said portion of the fuel body, to cool the gases and to condense the major portion of the tar-forming constituents of the said vapors, withdrawing cooled carbonized fuel from the lower part of said fuel body, mixing a minor portion of the carbonized fuel with bituminous fuel to form fresh fuel mixture, charging the mixture onto the upper part of said fuel body to maintain said fuel body, and rejecting the major portion of carbonized fuel withdrawn.

16. In the manufacture of coke and gas the process which comprises, producing a relatively long fuel body of mixed coal and coke in regulated proportions, said body being relatively cool at the charging end and at the withdrawal end, the proportion of coke in the said mixture being that required to prevent the formation of draft-obstructing aggregates through the caking of the coal of the said mixture and so to maintain the fuel body in a condition permitting free passage of the draft therethrough, advancing said fuel body through a comparatively long conduit, maintaining a carbonizing temperature in an intermediate localized carbonizing region of the fuel body to decompose bituminous matter of the fuel of said body, to form gas, condensable vapors and carbonized fuel, the said carbonizing temperature being maintained by introducing a limited and regulated quantity of combustion-supporting draft current sufficient for the stated purpose into the said fuel body in said carbonizing region, withdrawing gaseous bodies from said carbonizing region, conducting said gaseous bodies through the portion of the fuel body above said region in such manner that the fuel therein will be subjected to a gradually increasing temperature from the top to the lower part thereof while the gases and vapors will be subjected to a gradually decreasing temperature from the bottom to the top thereof, the temperature of the uncondensed gaseous bodies at the top of the said portion of said fuel body being maintained above 212° F. but below the condensing temperature of pitch, withdrawing cooled carbonized fuel from the lower part of said fuel body, mixing a regulated portion of carbonized fuel with bituminous fuel, charging the mixture onto the upper part of said fuel body and rejecting such portion of the carbonized fuel withdrawn as is not returned to said fuel body.

17. In the manufacture of coke and gas the process which comprises, producing a relatively long fuel body of mixed coal and coke in regulated proportions, said body being relatively cool at the charging end and

at the withdrawal end, the proportion of coke in the said mixture being that required to prevent the formation of draft-obstructing aggregates through the caking of the coal of said mixture and so to maintain the fuel body in a condition permitting free passage of the draft therethrough, advancing said fuel body through a comparatively long conduit, maintaining a carbonizing temperature in an intermediate carbonizing region of the fuel body to decompose bituminous matter of the fuel of said body, to form gas, condensable vapors and carbonized fuel, the said carbonizing temperature being maintained by introducing a limited and regulated quantity of combustion-supporting draft current sufficient for the stated purpose into the said fuel body in said carbonizing region, withdrawing gases and vapors from said carbonizing region through the portion of said fuel above said region to heat said portion of the fuel body, to cool the gases and to condense the major portion of the tar-forming constituents of the said vapors, the said gases and vapors being conducted through said portion of the fuel body in such manner that the fuel therein will be subjected to a gradual increase in temperature from the top to the lower part thereof while the gases and vapors will be subjected to a gradual decrease in temperature from the bottom to the top thereof, the temperature of the uncondensed gaseous bodies at the top of the said portion of said fuel body being maintained above the temperature at which water will be deposited but below the condensing temperature of pitch, carrying a portion of each of the several tar-forming constituents condensed back into a level in the said fuel body at which the temperature is sufficiently high to convert a substantial portion of that constituent into gas, withdrawing cooled carbonized fuel from the lower part of said fuel body, mixing a regulated portion of carbonized fuel with bituminous fuel, charging the mixture onto the upper part of said fuel body and rejecting such portion of the carbonized fuel withdrawn as is not returned to said fuel body.

18. In the manufacture of coke and gas the process which comprises, producing a relatively long fuel body of mixed coal and coke in regulated proportions, the proportion of coke in the said mixture being that required to prevent the formation of draft-obstructing aggregates through the caking of the coal of said mixture and so to maintain the fuel body in a condition permitting free passage of the draft therethrough, advancing said fuel body through a comparatively long conduit, maintaining a carbonizing temperature in an intermediate localized carbonizing region of the fuel body to decompose bituminous matter of the fuel of

said body, to form gas, condensable vapors and carbonized fuel, the said carbonizing temperature being maintained by introducing a limited and regulated quantity of 5 combustion-supporting draft current sufficient for the stated purpose into said fuel body in said carbonizing region, conducting the gases and vapors from said carbonizing region through the portion of said body 10 above said region to heat the said portion of the fuel body, to cool the said gases and to condense the major portion of the tar-forming constituents of the said gases and vapors, the said gases and vapors being conducted through said portion of said fuel body in such manner that the fuel therein will be subjected to a gradual increase in temperature from the top to the lower part thereof while the gases and vapors will be 15 subjected to a gradual decrease in temperature from the bottom to the top thereof, the temperature of the said gases at the top of the said portion of said fuel body being maintained above 212° F., withdrawing the 20 cooled gases from the upper part of said fuel body at a temperature above 212° F. but below the temperature of condensation of the heavy tarry matter of the draft current, withdrawing cooled carbonized fuel 25 from the lower part of said fuel body, mixing a minor portion of carbonized fuel with bituminous fuel to form fresh fuel mixture, charging the fuel mixture onto the upper part of said fuel body to maintain the same, 30 and rejecting the major portion of the carbonized fuel withdrawn.

19. In the manufacture of coke and gas the process which comprises, producing a relatively long fuel body of mixed coal and 40 coke in regulated proportions, said fuel body being relatively cool at the charging end and at the withdrawal end, the proportion of coke in the said mixture being that required to prevent the formation of draft-obstructing 45 aggregates through the caking of the coal of said mixture and so to maintain the fuel body in a condition permitting free passage of the draft therethrough, advancing said fuel body through a comparatively long 50 conduit, maintaining a carbonizing temperature in an intermediate localized carbonizing region of the fuel body to decompose bituminous matter of the fuel of said body, to form gas, condensable vapors and carbonized fuel, said carbonizing temperature being maintained by introducing a limited and regulated quantity of combustion-supporting 55 draft current sufficient for the stated purpose into the said fuel body in said carbonizing region and in part by returning to said region the major part of the heat carried out of the same, withdrawing gaseous bodies from said carbonizing region, conducting the said gaseous bodies through the 60 portion of the fuel body above said region 65

to heat said portion of the fuel body, to cool said gases and to condense the major portion of the tar-forming constituents of the said gaseous bodies, the said gases and vapors being conducted through said portion of the fuel body in such manner that the fuel therein will be subjected to a gradual increase in temperature from the top to the lower part thereof while the gases and vapors will be subjected to a gradual decrease in temperature from the bottom to the top thereof, the temperature of the said gases and vapors at the top of the said portion of said fuel body being maintained above 212° F. but below the temperature of 70 condensation of pitch, carrying a portion of each of the several constituents of the condensed tarry matter back into a level of the said fuel body at which the temperature is sufficiently high to convert a substantial portion of that constituent into gas, withdrawing gases from the upper part of said fuel body at a temperature above 212° F. but below the temperature of condensation of the tarry matter of the draft current, 75 passing the gases withdrawn through the heating passages of a heat transferring apparatus to evaporate water, contacting a relatively cool gaseous fluid with that portion of the said fuel body which has advanced beyond said carbonizing region to quench the carbonized fuel of said portion of said fuel body and to heat the said gaseous body, withdrawing cooled carbonized fuel from the lower part of said fuel 80 body, mixing a regulated portion of carbonized fuel with bituminous fuel, charging the mixture onto the upper part of said fuel body and rejecting such portion of the carbonized fuel withdrawn as is not returned to 85 said fuel body.

20. In the manufacture of coke and gas the process which comprises, producing a relatively long fuel body of mixed coal and coke in regulated proportions, said body being relatively cool at the charging end and at the withdrawal end, the proportion of coke in the said mixture being that required to prevent the formation of draft-obstructing 90 aggregates through the caking of the coal of said mixture and so to maintain the fuel body in a condition permitting free passage of the draft therethrough, advancing said fuel body through a comparatively long 95 conduit, said fuel body being advanced and maintained by withdrawing material from one end of said fuel body and charging fuel mixture onto the other end of said fuel body, maintaining a carbonizing temperature in an intermediate carbonizing 100 region of the fuel body to decompose bituminous matter of the fuel of said body, to form gas, condensable vapors and carbonized fuel, the said carbonizing temperature being maintained by introducing a limited 105

110

115

120

125

130

and regulated quantity of combustion-supporting draft current into the said fuel body in said carbonizing region, the quantity of combustion-supporting draft current introduced being regulated to that which will generate sufficient heat by the union of its combustion-supporting constituents with a portion of the combustible matter present in said carbonizing region to maintain the temperature required for the stated purpose, withdrawing gaseous bodies from said carbonizing region, conducting said gaseous bodies through the portion of said fuel body above said region to heat the said portion of the fuel body, to cool the said gaseous bodies and to condense the major part of the tar-forming constituents of said gaseous body, the said gaseous body being conducted through the said portion of the fuel body in such manner that the fuel therein will be subjected to a gradual increase in temperature from the top to the lower part thereof while the gases and vapors will be subjected to a gradual decrease in temperature from the bottom to the top thereof, the temperature of the gaseous body withdrawn at the top of said portion of said fuel body being maintained above 212° F. but below the temperature of condensation of pitch, carrying each of the several tar-forming constituents condensed back into a level in said fuel body at which the temperature is sufficiently high to convert a substantial portion of that constituent into gas, withdrawing uncondensed gases from said portion of said fuel body, passing the gases withdrawn through the heating passages of a heat transferring apparatus to evaporate water, removing illuminants and ammonia from a portion of the withdrawn gases, mixing water vapor with said portion of gases by conducting the said portion of gases through the heat receiving passages of said heat transferring apparatus in contact with the water which is being subjected to evaporation by heat abstracted from the withdrawn gases, the proportion of the water vapor formed to the said gases being that required to form a substantially saturated mixture at the temperature of said vapor, introducing the mixture of water vapor and gas into and passing the same through the carbonized fuel in the lower part of said fuel body to quench the said carbonized fuel and to heat the said mixture of gas and water vapor, the volume of the gas and water vapor being that required to cool said carbonized fuel to the desired degree.

21. In the manufacture of coke and gas the process which comprises, producing a relatively long fuel body of mixed coal and coke in regulated proportions, said fuel body being comparatively cool at the charging end and at the withdrawal end, advancing said fuel body through a relatively long conduit, said fuel body being advanced and

maintained by withdrawing material from one end of said fuel body and charging fuel mixture onto the other end of said fuel body, maintaining a carbonizing temperature in an intermediate localized carbonizing region of the fuel body to decompose bituminous matter of the fuel of said body, to form gas, condensable vapors and carbonized fuel, the said carbonizing temperature being maintained by introducing a limited and regulated quantity of combustion-supporting draft current sufficient for the stated purpose into said fuel body in said carbonizing region and in part by returning to said region the major part of the heat carried out of the same by the products of the carbonizing action, withdrawing gases from the upper part of said fuel body, contacting a relatively cool gaseous fluid with that portion of said fuel body which has advanced beyond the carbonizing region to quench the said carbonized fuel and to heat the said gaseous body, conducting the heated gaseous body into the carbonizing region, withdrawing cooled carbonized fuel from the lower part of said fuel body, mixing a regulated minor portion of carbonized fuel with bituminous fuel, charging the mixture onto the upper part of said fuel body and rejecting the major portion of the carbonized fuel withdrawn.

22. In the manufacture of coke and gas the process which comprises, producing a relatively long fuel body of mixed coal and coke in regulated proportions, said body being relatively cool at the charging end and at the withdrawal end, advancing said fuel body through a comparatively long conduit, maintaining a carbonizing temperature at an intermediate localized carbonizing region of the fuel body to decompose bituminous matter of the fuel of said body, to form gas, condensable vapors and carbonized fuel, the temperature of the said carbonizing region being maintained by introducing a limited and regulated quantity of combustion-supporting draft current into the said fuel body in said carbonizing region, the quantity of combustion-supporting draft current introduced being regulated to that which will generate the quantity of heat required for the stated purpose, contacting a relatively cool gaseous fluid with that portion of said fuel body which has advanced beyond said carbonizing region to quench the said carbonized fuel and to heat the said gaseous body, conducting the heated gaseous body into the said carbonizing region, withdrawing cooled carbonized fuel from the lower part of said fuel body, mixing a regulated portion of the carbonized fuel with bituminous fuel, charging the mixture onto the upper part of said fuel body and rejecting such portion of the carbonized fuel as is not returned to said fuel body.

23. In the manufacture of coke and gas the process which comprises, producing a relatively long fuel body of mixed coal and coke in regulated proportions, the proportion of coke in the said mixture being that required to prevent the formation of draft-obstructing aggregates through the caking of the coal of said mixture and so to maintain the fuel body in a condition permitting free passage of the draft therethrough, advancing said fuel body through a comparatively long conduit, maintaining a carbonizing temperature in an intermediate localized carbonizing region of the fuel body to decompose bituminous matter of the fuel of said body, to form gas, condensable vapors and carbonized fuel, the said carbonizing temperature being maintained by introducing a limited and regulated quantity of combustion-supporting draft current sufficient for the stated purpose into the said fuel body in said carbonizing region, conducting the gases and vapors from the said carbonizing region into and through that portion of the said fuel body above said region, the said gases and vapors being conducted through said portion of said fuel body in such manner that the fuel therein will be subjected to a gradual increase in temperature from the top to the lower part thereof while the gases and vapors will be subjected to a gradual decrease in temperature from the bottom to the top thereof, the temperature of the said gases and vapors at the top of said portion of said fuel body being maintained above 212° F. but below 300° F., whereby tar-forming constituents of the draft current passing through said portion of said fuel body will be condensed, carrying a portion of each of the several constituents of the condensed tarry matter back into a level in the said fuel body at which the temperature is sufficiently high to convert a substantial portion of that constituent into gas, withdrawing gases from the upper part of said fuel body, contacting a relatively cool gaseous fluid with that portion of said fuel body which has advanced beyond said carbonizing region to quench the carbonized fuel and to heat the said gaseous body, conducting the said gaseous fluid into the said carbonizing region, withdrawing cooled carbonized fuel from the lower part of the said fuel body, mixing a regulated portion of carbonized fuel with the bituminous fuel, charging the mixture onto the upper part of said fuel body and rejecting such portion of the carbonized fuel withdrawn as is not returned to said fuel body.

24. In the manufacture of coke and gas the process which comprises, producing a relatively long fuel body of mixed coal and coke in regulated proportions, said body being comparatively cool at the charging

end and at the withdrawal end, advancing said fuel body through a relatively long conduit, maintaining a carbonizing temperature in an intermediate localized carbonizing region of the fuel body to decompose bituminous matter of the fuel of said body to form gas, condensable vapors and carbonized fuel, said carbonizing temperature being maintained by introducing a limited and regulated quantity of combustion-supporting draft current into the said fuel body in said carbonizing region and in part by returning to said region the major part of the heat carried out of the same by the products of the carbonizing action, the quantity of combustion supporting draft current introduced being regulated to that which will generate sufficient heat by the union of its combustion-supporting constituents with a portion of the combustible matter present in said carbonizing region to make up any deficiency in the temperature of the fuel body in said region necessary for the stated purpose over that due to the sensible heat carried into the said region, conducting said gaseous bodies through that portion of the fuel body above said region in such manner that the fuel therein will be subjected to a gradual increase in temperature from the top to the lower part thereof while the said gases will be subjected to a gradual decrease in temperature from the bottom to the top thereof, the temperature of the said gases and vapors at the point of withdrawal from the said fuel body being maintained above 212° F. but below the temperature of condensation of pitch, withdrawing the so-cooled gases from said fuel body, mixing water vapor with a portion of the said gases, introducing the mixture of water vapor and gas into and passing the same through the carbonized fuel in the lower part of said fuel body to cool the said carbonized fuel and to heat the mixture of gas and water vapor, the volume of the gas and water vapor introduced being regulated to that required to quench said carbonized fuel, conducting the heated fluids into the said carbonizing region and mingling the same with the draft current passing through said region, withdrawing cooled carbonized fuel from the lower part of said fuel body, mixing a regulated portion of said carbonized fuel with bituminous fuel, charging the mixture onto the upper part of said fuel body and rejecting such portion of the carbonized fuel withdrawn as is not returned to said fuel body.

25. In the manufacture of coke and gas the process which comprises, producing a relatively long fuel body of mixed coal and coke in regulated proportions, the proportion of coke in the said mixture being that required to prevent the formation of draft-

obstructing aggregates through caking of the coal of said mixture and so to maintain the fuel body in a condition permitting free passage of the draft therethrough, said body being relatively cool at the charging end 5 and at the withdrawal end, maintaining a carbonizing temperature in an intermediate localized carbonizing region of the fuel body to decompose bituminous matter of the fuel of said body, to form gas, condensable vapors and carbonized fuel, the said carbonizing temperature being maintained by introducing a limited and regulated quantity of combustion-supporting draft current into the said fuel body in said carbonizing region, the quantity of combustion-supporting draft current introduced being regulated to that which will generate sufficient heat by the union of its combustion-supporting constituents with a portion of the combustible matter present in said carbonizing region to make up any deficiency in the temperature of the fuel body in said region, necessary for the stated purpose, conducting gases and vapors from said carbonizing region through the portion of the said fuel body above said region to heat the said portion of fuel body, to cool the gases and to condense condensable tarry vapors, withdrawing gas from the upper part of said fuel body at a temperature above 212° F. but below the temperature of condensation of the tarry matter of the draft current, passing the gas withdrawn through the 35 heating passages of a heat transferring apparatus to evaporate water, removing illuminants and ammonia from a portion of the withdrawn gas, mixing water vapor with the said portion of gas by conducting the said portion of gas through the heat-receiving passages of said heat-transferring apparatus in contact with water which is being subjected to evaporation by sensible heat abstracted from the withdrawn gases, the 40 proportion of water vapor formed to the said gas being that required to form a substantially saturated mixture at the temperature of said vapor, introducing the mixture of water vapor and gas into and passing the same through the carbonized fuel and 45 ash of the burned fuel in the lower part of said fuel body to quench the said carbonized fuel and ash and to heat the mixture of gas and water vapor, the volume of the gas and water vapor being regulated to that required to cool the said carbonized fuel and ash to the desired degree, and withdrawing cooled carbonized fuel and ash from the lower part of said fuel body.

26. In the manufacture of coke and gas the process which comprises, producing a relatively long fuel body of mixed coal and coke in regulated proportions, said fuel body being relatively cool at the charging end 50 and at the withdrawal end, maintaining a

carbonizing temperature in an intermediate localized carbonizing region of the fuel body to decompose bituminous matter of the fuel of said body, to form gas, condensable vapors and carbonized fuel, the said carbonizing temperature being maintained by introducing a limited and regulated quantity of combustion-supporting draft current into the said fuel body in said carbonizing region and in part by returning to said region the 70 major part of the heat carried out of the same by the products of the carbonizing action therein, the quantity of combustion-supporting draft current introduced being regulated to that which will generate sufficient heat by the union of its combustion-supporting constituents or constituent with a portion of the combustible matter present in said carbonizing region to make up any deficiency in the temperature of the fuel 75 body in said region for the stated purpose over that due to the sensible heat carried into said region, withdrawing gaseous bodies from said region, conducting gaseous bodies through that portion of the said fuel body above said carbonizing region in such manner that the fuel therein will be subjected to a gradual increase in temperature from the top to the lower part thereof, while the said gaseous bodies will be subjected to 80 a gradual decrease in temperature from the bottom to the top thereof, to condense tar-forming constituents from said gaseous bodies, carrying a portion of each of the several tar-forming constituents condensed back 85 into a level in the said fuel body at which the temperature is sufficiently high to convert a substantial portion of that constituent into gas, withdrawing gas from the upper part of said fuel body at a temperature 90 above 212° F. but below the temperature of condensation of the tarry matter of the draft current, mixing water vapor with a portion of the withdrawn gases, the proportion of water vapor being that required to 95 form a substantially saturated mixture, introducing the mixture of water vapor and gas into and passing the same through the carbonized fuel in the lower part of said fuel body to quench said carbonized fuel and to 100 heat the mixture of gas and water vapor, withdrawing cooled carbonized fuel mixed with the ash from said combustion from the lower part of said fuel body, separating coarse carbonized fuel from the mixture, 105 mixing a regulated portion of the coarse carbonized fuel with bituminous fuel, charging the mixture onto the upper part of said fuel body and rejecting the ash and such portion of the carbonized fuel withdrawn as is not 110 returned to said fuel body.

27. In the manufacture of coke and gas the process which comprises, producing a relatively long fuel body of mixed coal and coke in regulated proportions, said body be- 115

ing relatively cool at the charging end and at the withdrawal end, advancing said fuel body through a comparatively long conduit, maintaining a carbonizing temperature in an intermediate localized carbonizing region 5 of the said fuel body to decompose bituminous matter of the fuel of the said body, to form gas, condensable vapors and carbonized fuel, said carbonizing temperature being maintained by introducing a limited and regulated quantity of combustion-supporting draft current into the said fuel body in the said carbonizing region and in part by returning to said region the major part of 10 15 the heat carried out of the same, the quantity of combustion-supporting draft current introduced being regulated to that which will generate sufficient heat by the union of its combustion-supporting constituents with a portion of the combustible matter present 20 in said carbonizing region to make up any deficiency in the temperature of the fuel body in said region for the stated purpose over that due to the sensible heat carried 25 into the said region, withdrawing gases and vapors from said region, conducting the said gases and vapors through the portion of the fuel body above said region in such manner that the major portion of the sensible heat 30 carried by the said gases and vapors will be transferred to the fuel therein and the major portion of the tar-forming constituents of the vapors will be condensed withdrawing the cooled gas from the upper portion 35 of the said fuel body, passing the gas withdrawn through the heating passages of a heat transferring apparatus to evaporate water, removing illuminants and ammonia from a portion of the withdrawn gas, mixing the water vapor formed with said 40 portion of gas, the proportion of the water vapor formed to the said gas being that required to form a substantially saturated mixture at the temperature of said vapor, introducing the mixture of water vapor and 45 gas into and passing the same through the carbonized fuel and ash in the lower part of said fuel body to quench the said carbonized fuel and ash and to heat the mixture of gas and water vapor, and withdrawing cooled 50 carbonized fuel and ash from the lower part of the said fuel body.

28. In the manufacture of coke and gas the process which comprises, producing a 55 relatively long fuel body of mixed fuel and coke in regulated proportions, said fuel body being relatively cool at the charging end and at the withdrawal end, the proportion of coke in the said mixture being that required 60 to prevent the formation of draft-obstructing aggregates through the caking of the coal of said mixture and so to maintain the fuel body in a condition permitting free passage of the draft current therethrough, advancing the said fuel body through a com-

paratively long conduit, said fuel body being advanced and maintained by withdrawing material from one end of said fuel body and charging fuel mixture onto the other end of said fuel body, maintaining a carbonizing temperature in an intermediate localized carbonizing region of the fuel body to decompose bituminous matter of the fuel, to form gas, condensable vapors and carbonized fuel, the said carbonizing temperature being maintained by introducing a limited and regulated quantity of combustion-supporting draft current into said fuel body in said carbonizing region to burn a minor portion only of the fuel of said body to ash, conducting gases and vapors from said carbonizing region through the portion of said fuel body above said region to preheat the said portion of the fuel body and to cool the withdrawn gases and vapors to a temperature such as will condense substantially 80 all of the heavy tarry constituents of the said gases and vapors, said gases and vapors being conducted through the said portion of the fuel body in such manner that the fuel 85 therein will be subjected to a gradual increase in temperature from the top to the lower part thereof while the gases and vapors will be subjected to a gradual decrease in temperature from the bottom to the 90 top thereof, carrying a portion of each of the several constituents of the condensed tarry matter back into a level in said fuel body at which the temperature is sufficiently high to convert a substantial portion 95 of that constituent into gas, withdrawing gas from the upper part of said fuel body at a temperature above 212° F. but below the temperature of condensation of the tarry matter of the draft current, passing 100 the gas withdrawn through the heating passages of a heat transferring apparatus to evaporate water, removing illuminants and ammonia from a portion of the withdrawn gas, mixing water vapor with said portion 105 of gas by conducting the said portion of gas through the heat receiving passages of said heat transferring apparatus in contact with the water which is being subjected to evaporation by sensible heat abstracted from 110 the withdrawn gas, introducing the mixture of water vapor and gases into and passing the same through the carbonized fuel and ash in the lower part of said fuel body in such manner that the said carbonized fuel 115 and ash will be subjected to a gradual decrease in temperature as it advances toward the bottom of the said fuel body while the said mixture of water vapor and gas will be subjected to a gradual increase in temperature during its passage upward from the bottom of the said fuel body, the combined volume of the gas and water vapor being regulated to that required to cool the 120 said carbonized fuel and ash to the de- 125 130

sired degree, withdrawing cooled carbonized fuel and ash from the lower part of said fuel body, separating a portion of the coarse carbonized fuel from the rest of the mixture of carbonized fuel and ash, mixing a regulated portion of the coarse carbonized fuel with bituminous fuel, charging the mixture onto the upper part of said fuel body and rejecting such portion of the carbonized fuel as is not returned to said fuel body.

29. In the manufacture of coke and gas the process which comprises, producing a relatively long body of mixed coal and coke in regulated proportions, said fuel body being relatively cool at the charging end and at the withdrawal end, maintaining a carbonizing temperature in an intermediate localized carbonizing region of said fuel body to decompose bituminous matter of the fuel in the said body, to form gas, condensable vapors and carbonized fuel, said carbonizing temperature being maintained by introducing a limited and regulated quantity of combustion-supporting draft current into said body and by returning to said carbonizing region the major part of the heat carried out of the same by the products of the carbonization, the quantity of combustion-supporting draft current introduced being regulated to that which will generate sufficient heat by the union of its combustion-supporting constituents with a portion of the combustible matter present in said carbonizing region to make up any deficiency in the temperature of the fuel body in said region for the stated purpose over that due to the sensible heat carried into the said region, withdrawing gaseous bodies from said region, conducting the said gaseous bodies through the portion of said fuel body above said region, to preheat the said portion of the fuel body, to cool the gases and to condense substantially all of the heavy tarry constituents of the said gases, the said gases and vapors being conducted through said portion of said fuel body in such manner that the fuel therein will be subjected to a gradual increase in temperature from the top to the lower part thereof while the gases and vapors will be subjected to a gradual decrease in temperature from the top to the bottom thereof, withdrawing the uncondensed gases from the upper part of said fuel body at a temperature above 212° F. but below the temperature of condensation of the tarry matter of the draft current, removing illuminants and ammonia from a portion of the withdrawn gases, mixing a regulated portion of water vapor with the said portion of withdrawn gases the proportion of the water vapor mixed with the said gases being that required to form a substantially saturated mixture at the temperature of the said vapor, introducing the mixture of water

vapor and gas into and passing the same through the carbonized fuel in the lower part of said fuel body, to quench the said carbonized fuel and to heat the mixture of gas and water vapor, conducting the heated fluids into the said carbonizing region and mingling the same with the draft current of the said region, withdrawing cooled carbonized fuel from the lower part of said fuel body, mixing a regulated minor portion of carbonized fuel withdrawn with bituminous fuel, charging the mixture onto the upper part of said fuel body and rejecting the major portion of the carbonized fuel withdrawn.

30. In the manufacture of coke and gas the process which comprises, producing a relatively long body of mixed coal and coke in regulated proportions, said fuel body being relatively cool at the charging end and at the withdrawal end, the proportion of coke in the said mixture being that required to prevent the formation of draft-obstructing aggregates through the caking of the coal of said mixture and so to maintain the fuel body in a condition permitting free passage of the draft current therethrough, maintaining a carbonizing temperature in an intermediate localized carbonizing region of the fuel body to decompose bituminous matter of the fuel body, to form gas, condensable vapors and carbonized fuel, the said carbonizing temperature being maintained by introducing a limited and regulated quantity of combustion-supporting draft current into the said fuel body in said carbonizing region and by returning to said region the major part of the heat carried out of the same, the quantity of combustion-supporting draft current introduced being regulated to that which will generate sufficient heat by the union of its combustion-supporting constituents with a portion of the combustible matter present in said carbonizing region to make up any deficiency in the temperature of the fuel body in said region for the stated purpose over that due to the sensible heat carried into the said region, conducting gaseous bodies from said carbonizing region through the portion of said fuel body above said region of the fuel body to cool the said gases to a temperature such as will condense the major portion of the tar-forming constituents of the said gaseous bodies, the said gaseous bodies being conducted through said portion of the fuel body in such manner that the fuel therein will be subjected to a gradual increase in temperature from the top to the lower part thereof while the said gaseous bodies will be subjected to a gradual decrease in temperature from the bottom to the top thereof, carrying a portion of each of the several constituents of the condensed matter back into a level in said

fuel body at which the temperature is sufficiently high to convert a substantial portion of that constituent into gas, withdrawing the uncondensed portion of said gases from the upper part of said fuel body at a temperature above 212° F. but below the temperature of condensation of the tarry matter of the draft current, removing illuminants and ammonia from a portion of the withdrawn gases, mixing a regulated proportion of water vapor with the said portion of gases, the proportion of water vapor mixed with the said portion of gases being that required to form a substantially saturated mixture at the temperature of the said vapor, introducing the mixture of water vapor and gas into and passing the same through the carbonized fuel in the lower part of said fuel body to quench the said carbonized fuel and to heat the mixture of gas and water vapor, the volume of the said gas and water vapor being regulated to that required to cool said carbonized fuel to the desired degree, conducting the heated fluids into the said carbonizing region and mingling them with the gases generated in said region, withdrawing cooled carbonized fuel from the lower part of the said fuel body, mixing a regulated portion of carbonized fuel with bituminous fuel, charging the so-formed mixture onto the upper part of said fuel body and rejecting such portion of the carbonized fuel withdrawn as is not returned to said fuel body.

31. In the manufacture of coke and gas the process which comprises, producing a relatively long fuel body of mixed coal and coke in regulated proportions, said fuel body being relatively cool at the charging end and at the withdrawal end, maintaining a carbonizing temperature in an intermediate localized carbonizing region of the fuel body to decompose bituminous matter in the fuel of said body, to form gaseous bodies, the said carbonizing temperature being maintained by introducing a limited and regulated quantity of combustion-supporting draft current into the said fuel body in the said carbonizing region, the quantity of the combustion-supporting draft current introduced being regulated to that which will generate sufficient heat by the union of its combustion-supporting constituents with a portion of the combustible matter present in said carbonizing region to make up any deficiency in the temperature of the fuel body in said region for the stated purpose, withdrawing gaseous bodies from said carbonizing region, conducting said gaseous bodies through that portion of said fuel body which lies above said region to preheat the said portion of the fuel body and to cool the said gaseous bodies to that temperature at which the major part of the tar-forming constituents of the said gaseous

bodies will be condensed, withdrawing the uncondensed gaseous bodies from the upper part of said fuel body, passing the gas withdrawn through the heating passages of a heat transferring apparatus to evaporate water, removing illuminants and ammonia from a portion of the withdrawn gas, mixing water vapor with said portion of gas by conducting said portion of gas through the heat receiving passages of said heat transferring apparatus in contact with water which is being subjected to evaporation by sensible heat abstracted from the withdrawn gases, the proportion of the water vapor formed being that required to form a substantially saturated mixture at the temperature of said vapor, introducing the mixture of water vapor and gas into and passing the same through the carbonized fuel in the lower part of said fuel body to cool the said carbonized fuel and to heat the mixture of gas and water vapor, the combined volume of the said gas and water vapor being regulated to that required to quench the said carbonized fuel to the desired degree, withdrawing cooled carbonized fuel from the lower part of said fuel body, mixing a regulated proportion of carbonized fuel with bituminous fuel, charging the mixture onto the upper part of said fuel body and rejecting such portion of carbonized fuel withdrawn as is not returned to said fuel body.

32. In the manufacture of coke and gas the process which comprises, producing a relatively long fuel body of mixed coal and coke in regulated proportions, said fuel body being relatively cool at the charging end and at the withdrawal end, the proportion of coke in the said mixture being that required to prevent the formation of draft-obstructing aggregates through the caking of the coal of said mixture and so to maintain the fuel body in a condition permitting free passage of the draft current therethrough, maintaining a carbonizing temperature in an intermediate localized carbonizing region of the fuel body to form gas, condensable vapors and carbonized fuel, the said carbonizing temperature being maintained by introducing a limited and regulated quantity of combustion-supporting draft current into said fuel body sufficient to maintain such temperature and in part by returning to said region the major part of the heat carried out of the same by the products of the carbonizing action, withdrawing gaseous bodies from said region, conducting the said gaseous bodies through that portion of the said fuel body above said region to heat the said portion of the fuel body and to cool the said gaseous bodies to a temperature such as will condense the major portion of the tar-forming constituents of the said gaseous bodies, the said

gaseous bodies being contacted with said portion of said fuel body in such manner that the temperature of the gases at the top of said portion of said fuel body will be maintained above 212° F. but below the temperature of condensation of pitch, withdrawing gases from the upper part of said fuel body, passing the gases withdrawn through the heating passages of a heat transferring apparatus to evaporate water, removing the illuminants and ammonia from a portion of the withdrawn gases, mixing water vapor with said portion of said gases by conducting the said portion of gases through the heat receiving passages of said heat transferring apparatus in contact with water which is being subjected to evaporation by sensible heat abstracted from the withdrawn gases, introducing the mixture of water vapor and gas into and passing the same through the carbonized fuel in the lower part of said fuel body to quench the said carbonized fuel and to heat the mixture of gas and water vapor, the combined volume of the gas and water vapor being regulated to that required to cool the said carbonized fuel to the desired degree, withdrawing cooled carbonized fuel from the lower part of said fuel body, mixing a regulated portion of carbonized fuel with bituminous fuel and charging the mixture onto the upper part of said fuel body and rejecting such portion of carbonized fuel withdrawn as is not recharged to said fuel body.

33. In the manufacture of coke and gas the process which comprises, producing a relatively long fuel body of mixed coal and coke in regulated proportions, said body being relatively cool at the charging end and at the withdrawal end, maintaining a carbonizing temperature in an intermediate localized carbonizing region of the fuel body to decompose bituminous matter of the fuel of said body, to form gas, condensable vapors and carbonized fuel, the said carbonizing temperature being maintained by introducing a limited and regulated quantity of combustion-supporting draft current into the said fuel body in said carbonizing region and by returning to said region the major part of the heat carried out of the same, the quantity of combustion supporting draft current introduced being regulated to that which will generate sufficient heat by the union of its combustion-supporting constituents with a portion of the combustible matter present in said carbonizing region to make up any deficiency in the temperature of the fuel body in said region for the stated purpose over that due to the sensible heat carried into the said region, conducting gases and vapors from said carbonizing region through the portion of said fuel body above said region to heat the said

portion of the fuel body, to cool the gases and vapors and to condense the major part of the condensable vapors, the said gases and vapors being conducted through said portion of the fuel body in such manner that the fuel therein will be subjected to a gradual increase in temperature from the top to the lower part thereof while the gases and vapors will be subjected to a gradual decrease in temperature from the bottom to the top thereof, carrying a portion of each of the several constituents of the condensed matter back into a level in the said fuel body at which the temperature is sufficiently high to convert a substantial proportion of that constituent into gas, withdrawing the gases from the upper part of said fuel body at a temperature above 212° F. but below the temperature of condensation of the tarry matter of the draft current, mixing water vapor with a portion of the withdrawn gases, introducing the mixture of water vapor and gas into and passing the same through the carbonized fuel in the lower part of said fuel body, the combined volume of the gas and water vapor being regulated to that required to quench the said carbonized fuel to the desired degree, conducting the heated fluids into the carbonizing region, withdrawing cooled carbonized fuel from the lower part of said fuel body, mixing a regulated proportion of carbonized fuel with bituminous fuel, charging the mixture onto the upper part of said fuel body and rejecting such portion of the carbonized fuel withdrawn as is not returned to said fuel body.

34. In the manufacture of coke and gas the process which comprises, producing a relatively long fuel body of mixed bituminous coal and coke in regulated proportions, the proportion of coke in said mixture being that required to prevent the formation of draft-obstructing aggregates through the caking of the coal of said mixture and so to maintain the fuel body in a condition permitting free passage of the draft current therethrough, advancing said fuel body through a comparatively long conduit, the fuel body being advanced and maintained by withdrawing material from one end of said fuel body and charging fuel mixture onto the other end of said fuel body, maintaining a carbonizing temperature in an intermediate localized carbonizing region of the fuel body to decompose bituminous matter of the fuel of said body, to form gas, condensable vapors and carbonized fuel, the said carbonizing temperature being maintained by introducing a limited and regulated quantity of combustion-supporting draft current into the said fuel body in said carbonizing region and by returning to said carbonizing region the major part of the heat carried out of the same, the quantity

of combustion-supporting draft current introduced being regulated to that which will generate sufficient heat by the union of its combustion-supporting constituents with a portion of the combustible matter present in said carbonizing region to make up any deficiency in the temperature of the fuel body in said region for the stated purpose over that due to the sensible heat carried into said region, withdrawing from said region the gases and vapors formed therein, conducting said gases and vapors through a portion of said fuel body above said region to heat the said portion of the fuel body, to cool the gases and vapors and to condense the major part of the condensable vapors, the said gases and vapors being conducted through said portion of the fuel body in such manner that the fuel therein will be subjected to a gradual increase in temperature from the top to the lower part thereof while the gases and vapors will be subjected to a gradual decrease in temperature from the bottom to the top thereof, the temperature of the said gases and vapors at the top of the said portion of said fuel body being maintained above 212° F. but below 300° F., carrying a portion of each of the several constituents of the condensed matter back into a level in the said fuel body at which the temperature is sufficiently high to convert a substantial portion of that constituent into gas, withdrawing gas from the upper part of said fuel body at a temperature above 212° F. but below the temperature of condensation of the tarry matter of the draft current, passing the gas withdrawn through the heating passages of a heat transferring apparatus to evaporate water, re-

moving illuminants and ammonia from a portion of the withdrawn gas, mixing water vapor with said portion of gas by conducting said portion of gas through the heat receiving passages of said heat transferring apparatus in contact with the water which is being subjected to evaporation by sensible heat abstracted from the withdrawn gas, the proportion of the water vapor formed to the said gas being that required to form a substantially saturated mixture at the temperature of said vapor, introducing the mixture of water vapor and gas into and passing the same through the carbonized fuel in the lower part of said fuel body to quench the said carbonized fuel and to heat the mixture of gas and water vapor, the combined volume of the gas and water vapor being regulated to that required to cool the said carbonized fuel to the desired degree, conducting the heated fluids into said carbonizing region and mingling them with the gases evolved in said carbonizing region, withdrawing cooled carbonized fuel from the lower part of said fuel body, mixing with a regulated minor portion of carbonized fuel a quantity of bituminous fuel, charging the mixture onto the upper part of said fuel body to maintain said body, and rejecting such portion of carbonized fuel withdrawn as is not returned to said fuel body.

Signed at New York city in the county of New York and State of New York this 14th day of November A. D. 1911.

HENRY L. DOHERTY.

Witnesses:

FRANK L. BLACKBURN,  
H. A. MACKENZIE.

Copies of this patent may be obtained for five cents each, by addressing the "Commissioner of Patents, Washington, D. C."